

H. C. & E. A. COLBURN.  
ORE FLOTATION PROCESS.  
APPLICATION FILED MAY 31, 1916.

1,226,062.

Patented May 15, 1917.

2 SHEETS—SHEET 1.



H. C. & E. A. COLBURN.  
ORE FLOTATION PROCESS.  
APPLICATION FILED MAY 31, 1916.

1,226,062.

Patented May 15, 1917.

2 SHEETS—SHEET 2.



WITNESSES, Fig. 4  
F. H. Cuno.  
L. Rhoads.

INVENTORS  
H. C. COLBURN  
AND E. A. COLBURN.  
BY   
ATTORNEY.

# UNITED STATES PATENT OFFICE.

HERBERT C. COLBURN, OF COLORADO SPRINGS, AND ERNEST A. COLBURN, OF DENVER,  
COLORADO.

## ORE-FLOTATION PROCESS.

1,226,062.

Specification of Letters Patent. Patented May 15, 1917.

Application filed May 31, 1916. Serial No. 100,947. REISSUED

To all whom it may concern:

Be it known that we, HERBERT C. COLBURN and ERNEST A. COLBURN, citizens of the United States of America, residing, respectively, at Colorado Springs, in the county of El Paso, State of Colorado, and at Denver, in the county of Denver and State of Colorado, have invented certain new and useful Improvements in Ore-Flotation Processes, of which the following is a specification.

Our invention relates to improvements in the ore concentration process commonly known as the "flotation process," and its primary object resides in providing a novel method of separating the valuable mineral particles in finely divided ores by the production of a froth in which said particles are entrapped, exclusive of the gangue or worthless matter with which they were associated.

Our improved process consists in intermixing the finely divided ore with a liquid and a substance having a selective affinity for the valuable particles and subjecting this mixture together with air or other gas to violent agitation in a partial vacuum.

The vacuum expands the envelopes of gas and colloidal matter which are broken up by a constant bombardment of the particles on the parts of a mechanical agitator.

The bared sulfids are immediately coated with oil and the solid particles or the ore are thoroughly intermixed with the air and are in this condition discharged into a settling chamber in which the mixture is brought to a comparative condition of rest under atmospheric pressure.

As a result of these conditions the oil-coated particles rise naturally and easily to the surface, while the gangue settles to the bottom of the vessel and is drawn off. The air or other gas mixed with the solids also rises to the surface in a multitude of small bubbles and congregates with the oil into a heavy tenacious froth in which the valuable mineral particles are entrapped.

We are aware that apparatus have been devised in which ore-pulp, oil and air are intermixed by being drawn through a suction pump which delivers the mixture into the settling chamber, and it should be un-

derstood that the action to which the materials are subjected in an apparatus of this character differs widely from that which produces the perfect intermixture obtained in the practice of our improved method of emulsification.

In this method the pulp is, as before explained, intermixed with oil and air in a partial vacuum and instead of being rapidly circulated through the chamber in which the intermixture takes place, as in the pumping system hereinbefore referred to, it is retained in the mixing chamber until a thorough intermixture of the materials is obtained.

Without limiting ourselves to the employment of any particular apparatus for effecting the intermixture of the materials, we prefer to use, by reason of the simplicity of its construction, a chamber in which an agitating element has a rotary movement and which has an inlet of at most one-fourth the area of its outlet.

By the difference in sizes of the ingress and egress openings, a partial vacuum is constantly maintained in the mixing chamber while the rotating element impregnates the ore-pulp with oil and air admitted to the chamber through the openings the flow through which may be controlled by automatically regulated valves.

The intake opening of the chamber connects with a supply of ore sufficiently elevated to produce a head which feeds the material through the system in ratio to the discharge of the separated substances, and the outlet opening of the chamber connects with a spitzkasten which has an overflow for the froth and values in suspension and an outlet for the settling less valuable matter.

If so desired, a number of mixing chambers and spitzkastens may be connected in a series for the repeated treatment of settling matter.

An embodiment of our invention has been illustrated in the accompanying drawings in the various views of which like parts are similarly designated and in which,

Figure 1 represents a sectional elevation of a succession of units constructed in accordance with our invention and coöper-

atively combined for the repeated treatment of the pulp,

Fig. 2, an axial section through one of the mixing chambers shown in Fig. 1, taken 5 along the line 2—2,

Fig. 3, a section along the line 3—3, Fig. 2,

Fig. 4, a section similar to that shown in Fig. 2, showing a modified construction of 10 the agitating element with the mixing chamber,

Fig. 5, a section taken along the line 5—5, Fig. 4, and

Fig. 6, a sectional elevation showing a 15 modified method of producing a partial vacuum in the mixing chamber.

Referring first to Fig. 1 of the drawings, 20 2 designates a spitzkasten which has at its upper end an overflow 3 for the froth produced in the flotation process, and adjacent its bottom an outlet 4 for settling matter.

The reference numeral 5 designates a mixing chamber provided with an inlet which by means of a conduit 6 is connected with 25 an elevated source of ore supply 7, and with an outlet of comparatively large diameter which connects with a conduit 8 extending into the spitzkasten for the discharge of the material thereinto.

30 A rotary skimmer 9 mounted adjacent the overflow assists the movement of the supernatant froth into a laundry 10.

In the construction shown in the drawings, 35 a second mixing chamber 12 and a second spitzkasten 13 are operatively connected with the first described devices for the repeated treatment of the matter discharged through the outlet 4 of the first settling chamber.

40 The outlet 4 is to this end connected with the intake pipe 14 of the second mixing chamber and the outlet of the latter connects with a conduit 15 which discharges into the second spitzkasten 13.

45 The material settling in the last-mentioned chamber is discharged through a valve-controlled outlet 16 at the bottom thereof.

In this connection we desire it understood that a repeated treatment of the ore is required only under unusual circumstances 50 and that in most cases a single treatment of the ore is sufficient to extract practically all the values it contains.

The two spitzkastens shown in Fig. 1 are 55 connected by a conduit 17 for maintaining their liquid contents on an even level.

Now, referring to Figs. 2 and 3 of the drawings, the mixing chamber 5 is composed of a cylindrical casing 20 which has at its 60 upper end a tangentially disposed outlet-opening 18 and in one of its sides a central inlet opening 19.

The last mentioned opening connects with a nozzle 21 the cross-sectional area of which 65 is less than one-fourth the area of the outlet

opening and to which is attached the conduit 6 shown in Fig. 1.

The nozzle has an opening 22 for the admission of air, and a second opening 23 for the inlet of oil. The flow through the air 70 opening is controlled by a valve 24 which is yieldingly held upon its seat against atmospheric pressure, by a spring 25.

The flow of oil through the opening 23 is controlled by a needle valve 26 which opens 75 and closes the outlet of a branch 27 which connects with a conveniently located source of oil supply, and the two valves are connected for synchronous movement by means of a lever 28.

It will be seen that in the operation, air is admitted past the valve 24 while at the same time a proportionate quantity of oil is introduced into the material passing through the nozzle, through the opening 23.

80 The spring 25 is made of sufficient strength to maintain the vacuum in the mixing chamber, constantly at a predetermined pressure.

The casing 20 has at its opposite sides, centrally disposed, axially alined stuffing boxes 90 29 through which passes a shaft 30 which imparts a rotary movement to the mixing element within the chamber 5.

This element consists in the construction shown in Figs. 2 and 3, of a member 34 95 which is composed of a disk 31 fixed on the shaft adjacent a side of the chamber, and provided with a plurality of radially extending vanes 32 which at their outer ends are connected by a circumferential flange 33.

A second member 35 which in construction 100 is identical to the before described member 34, is fixed in the casing against the opposite side of the chamber 5, and the two opposed members coöperate to thoroughly intermix the materials introduced into the chamber, by a rapid rotary motion of the one with relation to the other.

The device shown in Figs. 3 and 4, differs 105 from the previously described form, only in the construction of the coöperative members of the mixing element.

The member mounted on the shaft 30 consists in this form of a disk 36 and a series of radial vanes 37 which in their outer longitudinal edges, have recesses 38 to admit correspondingly formed tongues 39 on the fixed member 40 at the opposite side of the chamber.

110 During rotation of the shaft these tongues pass through the recesses of the rapidly rotating element and thereby assist in effecting a thorough intermixture and comminution of the materials.

115 From the before going description the operation of our invention will be readily understood.

The ore entering the mixing chamber through its inlet, is thoroughly impregnated with the oil and air entering the nozzle 120

zle 21 through the openings 22 and 23, in a partial vacuum resulting from the difference in the areas of the inlet and outlet openings.

The partial vacuum in the mixing chamber expands the envelops of gas and colloidal matter which are subsequently broken by contact with the blades of the mechanical mixer.

The consequently bared sulfid particles 10 are immediately coated with oil and the solid constituents of the pulp including the gangue or worthless matter from which the sulfids are separated, are thoroughly intermixed with the air or other gas which is 15 atomized by the partial vacuum maintained in the mixing chamber.

The partial vacuum also expands and dissipates the gases present in the ore and thereby removes one of the chief causes for 20 failure in many of the flotation processes at present in use, it being well known that gases in ore-pulp float the gangue and thus oppose a clean separation.

The mixture discharged from the mixing 25 chamber enters the spitzkasten in which it is brought to a comparative condition of rest and in which the coated sulfid particles and atomized air rise to the surface where they congregate into a heavy tenacious froth, in 30 which the values contained in the ore are entrapped.

The froth is removed from the surface of the material through the overflow and the gangue or worthless matter settling in the 35 bottom of the chamber is discharged through the outlet 16.

The settling material may be conveyed to the dump or conducted to a second mixing chamber and a second spitzkasten as the circumstances and the character of the ore may 40 require.

In the construction shown in Fig. 6, a mixing chamber 41 is connected by means of a conduit 42 with a reservoir 43 in which 45 a vacuum of determinate pressure is maintained by a suction pump 44.

The mixing element in this form of our invention consists of a series of paddles 45 which radiate from a rotary vertical shaft 50 46.

In the operation of the modified form of our invention a partial vacuum is maintained in the reservoir 43 and the therewith communicating chamber 41 by the action of 55 the vacuum pump 44.

The pulp, oil and air entering the chamber are thoroughly intermixed by the rotary

movement of the blades 45 on the shaft 46 it being observed that as in the operation of the first-described apparatus, the gaseous envelops and colloidal matter are broken up by the partial vacuum, and a fine intermixture of the different substances is obtained, which results in a product consisting of the sulfid particles of ore coated with oil, the 60 gangue from which the coated particles are cleanly divided, and air which is thoroughly atomized throughout the finely divided mass.

The advantages of our improved method 70 of producing the froth in a flotation ore separating process, have been fully discussed in the first part of this description, and it is only necessary to add that by the automatic regulation of the air and oil 75 supply through the medium of the connected valves, the apparatus may be operated without requiring the constant attention of expert operators and that by reason of the comminution of the ore and its 80 thorough intermixture with the air and oil in a finely divided state, any oil or grease which otherwise would be unsuited for the purpose, may be employed to produce a froth of the desired tenacity. 85

Having thus described our invention, what we claim and desire to secure by Letters-Patent is:

1. The process of separating valuable particles of finely divided ores, consisting in 90 mixing ore-pulp with a substance having a selective affinity for the desired valuable particles, agitating and emulsifying the mixture with the addition of a gas, under a pressure less than atmospheric, and then 95 conducting the emulsified mixture to a separate receptacle in which the froth can rise under a higher pressure.

2. The process of separating valuable particles of finely divided ores, consisting in 100 mixing ore-pulp and oil, agitating and emulsifying the mixture with the addition of a gas, under a pressure less than atmospheric, and then conducting the emulsified mixture to a separate receptacle in which 105 the froth can rise under a higher pressure.

In testimony whereof we have affixed our signatures in presence of two witnesses.

HERBERT C. COLBURN.  
ERNEST A. COLBURN.

Witnesses:

G. J. ROLLANDET,  
L. RHOADES.